

## UNITED STATES PATENT OFFICE

2,221,256

## MAGNESIUM BASE ALLOY

John C. McDonald, Midland, Mich., assignor to  
The Dow Chemical Company, Midland, Mich., a  
corporation of Michigan

No Drawing. Application November 13, 1939,  
Serial No. 304,133

3 Claims. (Cl. 75—168)

The invention relates to magnesium base alloys. It more particularly concerns alloys of this nature having a high degree of formability, associated with other improved physical properties, such as increased tensile and yield strengths.

Magnesium alloys are being widely used in various structural and mechanical arts where a light weight metal is highly desirable, such as for use in making castings, forgings, and the like. However, the use of these alloys in the rolled form to make sheet metal articles requiring forming operations, such as bending, drawing, and the like, has not progressed as rapidly due to the fact that, in general, alloys having good formability, 10 permitting relatively sharp bends to be made without the articles developing external cracks, usually have inferior strength characteristics.

It is, accordingly, the principal object of the invention to provide a magnesium base alloy 20 which can be made into a rolled sheet or the like, possessing sufficient ductility or formability to be sharply bent, drawn, or otherwise shaped, while having improved tensile and yield strengths.

Other objects and advantages will be apparent 25 as the description of the invention proceeds.

My invention resides in the discovery that a magnesium base alloy composed of from 0.5 to 10 per cent of silver, 0.05 to 1 per cent of calcium, 1

ly high tensile strength and yield strength, is obtained when the alloy contains from 0.5 to 5 per cent of silver, 0.1 to 0.3 per cent of calcium, 6 to 12 per cent of cadmium, and from 0.5 to 5 per cent of zinc.

The specific proportion of each alloying metal and the total amount of the added alloying metals to be employed in the new alloy depends upon the use for which the alloy is intended. In general it is preferable to use alloys containing more 10 than about 80 per cent magnesium and less than 20 per cent of the added metals. For example, in alloys where a high ductility or formability associated with high yield and tensile strengths is of principal importance, the total added metals 15 should not materially exceed about 7 per cent; while in those instances where exceptionally high yield and tensile strengths are desirable, the percentage of total added metals should be above 20 about 12 per cent.

The following table, which lists some of the properties of rolled sheet metal made from my new alloy, as well as the properties of rolled sheet metal made from related quaternary alloys, 25 illustrates the improvement in strength characteristics of the new alloy over that of some of the closely related alloys. In the table, the per cent elongation is to be regarded as a measure of the ductility of the specimen.

Table

| Nominal composition in per cent (remainder=magnesium) |     |     |     | Annealed                       |                                  |                                | Cold rolled                    |                                  |                                |
|-------------------------------------------------------|-----|-----|-----|--------------------------------|----------------------------------|--------------------------------|--------------------------------|----------------------------------|--------------------------------|
| Ag                                                    | Ca  | Zn  | Od  | Yield strength in lbs./sq. in. | Tensile strength in lbs./sq. in. | Percent elongation in 2 inches | Yield strength in lbs./sq. in. | Tensile strength in lbs./sq. in. | Percent elongation in 2 inches |
| 0.9                                                   | 0.3 | 0.9 | 5.0 | 28,000                         | 38,000                           | 17                             | 45,000                         | 52,000                           | 5                              |
| 0.9                                                   | 0.3 | 0.9 | 5.0 | 18,000                         | 32,000                           | 20                             | 38,000                         | 42,000                           | 2                              |
| 0.8                                                   | 0.3 | —   | 5.1 | 22,000                         | 38,000                           | 20                             | 38,000                         | 46,000                           | 3                              |
| 0.9                                                   | 0.3 | 0.9 | 4.7 | 30,000                         | 41,000                           | 19                             | 44,000                         | 50,000                           | 2                              |
| 4.7                                                   | 0.3 | 2.5 | —   | 20,000                         | 38,000                           | 13                             | 46,000                         | 52,000                           | 4                              |
| 4.6                                                   | 0.3 | 2.5 | —   | 19,000                         | 39,000                           | 19                             | 46,000                         | 53,000                           | 3                              |
| 5.2                                                   | 0.3 | 2.5 | 5.4 | 23,000                         | 41,000                           | 16                             | 48,000                         | 55,000                           | 3                              |

to 15 per cent of cadmium, and from 0.1 to 10 per cent of zinc, the balance being substantially all magnesium, is endowed with the aforementioned properties. While the properties of good formability or ductility, associated with high tensile and yield strengths, are manifest over the entire range of composition indicated, I have found that, in general, the preferred combination of properties, such as the most desirable ductility for forming operations, coupled with exceptional

The properties listed in the above table under the section headed by the term "annealed" were obtained by first rolling the alloys at a temperature between about 500° to 600° F., and thereafter annealing them at various temperatures through 50 a temperature range of from 400° to 800° F. The properties selected for the table were those of the annealed specimens which exhibited the maximum elongation. The properties listed under the section headed "cold rolled" were obtained by

subjecting specimens of the alloys which had been hot rolled at a temperature of from 500° to 600° F. to additional rolling in the cold state to bring about a total reduction in thickness of from 2 to 5 per cent. The properties selected for the table were those of the cold rolled specimens which showed the greatest tensile and yield strengths, while having at least a 1 per cent elongation in 2 inches.

10 By comparison of the properties listed in the above table, it will be observed that the combined properties of my new polynary alloy are superior to those of the parent quaternary alloys having a similar percentage of alloying ingredients. For example, it will be noted that the compositions containing the lower percentages of alloying ingredients have greatly improved elongation, coupled with superior yield and tensile properties in the annealed state, while those having the higher percentages of the alloying ingredients show superior strength characteristics in the cold rolled state. Similar improvement will be noted throughout the range of the alloying ingredients indicated.

15 20 25 While the new alloy is most useful in wrought form, such as sheets, due to its formability characteristics, it may also be suitably used in making castings, forgings, extruded forms, and the like. It is further pointed out that my new alloy is amenable to solution and precipitation heat treatments, which, accordingly, modify its properties.

The new alloy may be compounded in any of the ways known to the art, such as by adding the ingredients to molten magnesium under suitable flux. The flux should be substantially free from magnesium chloride if the calcium content of the alloy is to be above 0.3 per cent. In those instances where an alloy is to be compounded containing less than 0.3 per cent of calcium, magnesium chloride may be present in the flux without exerting undue deleterious effects, but in this case it is usually preferable to add the calcium last and without too much stirring or agitation in order that the loss of calcium into the flux will be substantially prevented.

I claim:

1. A magnesium base alloy containing from 0.5 to 10 per cent of silver, 0.05 to 1 per cent of calcium, 1 to 15 per cent of cadmium, and from 0.1 to 10 per cent of zinc, the balance being magnesium.

2. A magnesium base alloy containing from 0.5 to 5 per cent of silver, from 0.1 to 0.3 per cent of calcium, from 6 to 12 per cent of cadmium, and from 0.5 to 5 per cent of zinc, the balance being magnesium.

3. A magnesium base alloy containing from 1 to 5 per cent of silver, from 0.1 to 0.3 per cent of calcium, from 6 to 8 per cent of cadmium, and from 1 to 5 per cent of zinc, the balance being magnesium.

JOHN C. McDONALD.

15

20

25

30